

## UNITED STATES PATENT OFFICE.

MELVIN M. GOLDSMITH, OF CHICAGO, ILLINOIS, ASSIGNOR OF ONE-HALF, BY MESNE ASSIGNMENTS TO GOLDSMITH BROS. SMELTING & REFINING COMPANY, OF CHICAGO, ILLINOIS, A CORPORATION OF WEST VIRGINIA.

## ALLOY FOR PEN POINTS.

No Drawing.

Application filed November 16, 1923. Serial No. 675,221.

*To all whom it may concern:*

Be it known that I, MELVIN M. GOLDSMITH, a citizen of the United States of America, and a resident of Chicago, in the county of Cook and State of Illinois, have invented a new and useful Improvement in Alloys for Pen Points, of which the following is a specification.

The main objects of this invention are to provide an osmium alloy which will have the hardness and acid resisting characteristics of the native alloy (osmium iridium) without the attendant losses which occur when the native alloy is used in the arts; and to provide an osmium alloy which can be economically worked; to provide an alloy with maximum wearing ability; to provide an alloy which is comparatively easy to use and to work; to provide an alloy which will retain the hardness and wearing properties of the native alloy osmiridium or iridosmium; to provide an alloy which is fusible with great difficulty and which can be gold soldered or frozen; to provide an alloy having a melting point between that of ruthenium and gold; to provide an alloy adapted to be worked in an electric furnace which will have more tenacity, uniformity of texture, and retain the hardness of the native alloy; to provide an alloy, which, when crushed or stamped, will not powder but will give particles approximately of cubical form.

In making the alloy the best results have been obtained when iridium, which occurs in the native alloy, is left out of the mixture and there is substituted from 10 to 20 per cent of ruthenium, another tetrad metallic element, which, next to osmium, is the most refractory. The melting point of the alloy is further reduced and the tenacity texture is found to be improved when from 3 to 10 per cent of the mixture is made up of one of the lighter metals, nickel, silver, or the like.

The operation of manufacture of alloys of this class comprises placing the metals in proper proportions in an electric furnace. After fusion the alloy button is stamped, cracked or crushed to obtain pieces which weigh approximately one-tenth of a grain each. All pieces which are smaller or are irregular in shape have to be discarded and are lost. Since the basic metals are rare

and expensive this loss is a very serious one. 55 The properly shaped and sized pieces are adapted to freezing on and finishing as pen tips and similar wearing surfaces. My discovery or invention comprises a new osmium alloy which hangs together when crushed, 60 does not powder, and which is uniform in texture; at the same time the new alloy has the wearing qualities of the native osmiridium.

In the arts the native alloy osmiridium 65 is known to be the most infusible alloy, at the same time the hardest. It will stand the greatest wear of any known substance. One of the uses is the fusing, soldering, or freezing of a small piece on the tip of a pen 70 to take the wear. The native alloy is very expensive and the preparation of the tip point is both difficult and expensive because of a large amount of waste which occurs when the native alloy is cracked or broken 75 into commercial tips. This waste comes from two sources; first, the native alloy when crushed or cracked, is prone to divide into small particles, too small to be used, sizes weighing less than one-tenth of a grain 80 each and irregular pieces are lost.

I claim:

1. An osmium alloy comprising 10 to 20 per cent of ruthenium, 3 to 10 per cent of nickel, and the rest osmium, 65 to 85 per 85 cent.

2. As a substitute for osmiridium, an osmium alloy containing twenty or more per cent of osmium, ten or more per cent of ruthenium and a small proportion of nickel 90 relative to the ruthenium.

3. An osmium alloy comprising osmium, 65 to 85 per cent, ruthenium, 10 to 20 per cent, and a tetrad metal flux, 3 to 10 per 95 cent.

4. An osmium alloy suitable for forming the metal wearing surface of pen tips, comprising ruthenium in excess of the amount of osmium present.

5. As a substitute for osmiridium, a hard 100 alloy adapted to provide a durable wearing surface and comprising osmium combined with ruthenium in the same proportion in which iridium occurs in the natural native alloy osmiridium. 105

Signed at Chicago this 13th day of November 1923.

MELVIN M. GOLDSMITH.